

1

3,443,976

## MINERAL GRINDING AIDS

Vance H. Dodson, Needham, and Frank G. Serafin, Peabody, Mass., assignors to W. R. Grace & Co., Cambridge, Mass., a corporation of Connecticut  
No Drawing. Filed Oct. 14, 1965, Ser. No. 496,144  
Int. Cl. C04b 7/52

U.S. Cl. 106—90

3 Claims

## ABSTRACT OF THE DISCLOSURE

In the grinding of minerals (e.g., Portland cement) an additive which can be morpholine, N-methylmorpholine or a byproduct from the continuous commercial production of heterocyclic amines consisting predominantly of 4-(2-aminoethoxy) ethylmorpholine, 2-(4-morpholethoxy) ethanol, and bis-2-(4-morpholiny) ethyl ether is added to increase the efficiency of the grinding operation.

This invention relates to grinding minerals, and more particularly to the use of an additive for improving the efficiency in grinding minerals and improving the pack set characteristics of minerals.

At some stage in the processing of minerals, a grinding operation is generally necessary in order to reduce the particular mineral to a relatively small particle size. It is desirable in this grinding step to have as efficient an operation as possible, that is, to reduce the mineral to the desired particle size at a relatively rapid rate.

A grinding aid is employed to promote an increase in efficiency, either by increasing the rate of production or by increasing the fineness of the particles at the same rate of production without having adverse effects on any of the properties of the ground product.

Cleavage of the particles during grinding of the minerals exposes fresh or nascent surfaces which have high energies due, probably, to the breaking of ionic bonds. The surface forces of the ground particles persist for some time after grinding and lead to compaction or pack set and/or poor fluidity if they are not reduced. Mineral particles when compacted by vibration; e.g., when transported in a hopper car, often become semi-rigid and will not flow until considerable mechanical effort has been applied to break up the compaction. On the other hand, undue reduction or the complete absence of surface forces is undesirable because the finely ground mineral becomes excessively fluid.

The term "pack set" as used herein is intended to refer to the agglomeration or adhesion of particles by, e.g., storing or transporting in bulk. Adhesion results from surface forces, the majority of which are created during the grinding of the minerals. "Pack set index" is a relative term which numerically indicates how prone a particular material is to start flowing after it is stored or transported in bulk. "Pack set index ratio" is the relative pack set index of the untreated sample compared to the treated sample. This ratio is used to permit comparison between different samples of the mineral.

Pack set index is determined in the following manner: 100 grams of the mineral is placed in a 250 milliliter Erlenmeyer flask set on top of a variable vibrator. The flask containing a mineral is vibrated 15 seconds after which time it is removed from the vibrator and fed into a jig with the axis of the flask lying horizontally. The flask is then rotated about its axis until the mineral which is compacted on the bottom of the flask collapses. The flask is twisted by turning at 180° angles at approximately 100 twists per minute. The number of 180° twists required for the mineral sample to collapse establishes the pack set

2

index. Thus, the greater the energy requirement to break up the bed, the higher will be the pack set index.

An additive has now been found which will function as a grinding aid and a pack set inhibitor for minerals. The novel additive of the present invention may be represented by the formulae:



and



wherein  $\text{R}^1$  is an alkaryl or aryl radical;  $\text{R}^2$  is hydrogen or an alkyl radical;  $\text{R}^3$  is hydrogen, hydroxyl, alkyl or aryl radical;  $\text{R}^5$  is hydrogen, alkyl, alkoxy or alkylhydroxy radical;



is pyrrolidyl, pyrrolyl, morpholinyl, morpholino or piperidyl radicals;  $\text{Y}$  is pyridyl, piperadyl, pyrimidinyl and pyradazinyl;  $\text{R}^6$  is halogen, hydroxy or an alkyl radical; and  $n$  is an integer from 0 to 5, inclusive.

$\text{R}^1$  is preferably alkylphenyl or phenyl radical. It should also be understood that the aryl radical may contain substituents such as halogen, e.g., chlorine and bromine, alkyl, amino or hydroxyl radicals. The alkyl groups represented by  $\text{R}^2$ ,  $\text{R}^3$ ,  $\text{R}^5$ , and  $\text{R}^6$  are preferably lower alkyl, i.e., 1 to 6 carbon atom alkyl radicals. The terms pyrrolyl, pyrrolidyl, morpholino, morpholinyl and piperadyl, as used therein are intended to include the substituted radicals which are known to the art, e.g., N-methylmorpholino, and 4-(2-aminoethoxy) ethylmorpholine.

The additives of Formulae B and C are particularly preferred because of the particularly advantageous pack set properties as well as the increased grinding efficiency achieved with these classes of materials.

As illustrative of additives within the scope of the present invention, mention may be made of the following:

|                       |                      |
|-----------------------|----------------------|
| Aniline               | Piperidine           |
| p-toluidine           | Pyrrole              |
| M-phenylenediamine    | Pyrroline            |
| Dimethylaniline       | Pyrrolidine          |
| Diphenylamine         | Pyridazine           |
| 2,4,6-tribromoaniline | Pyrimidine           |
| N-phenylhydroxylamine | N-methylmorpholine   |
| Beta-phenethylamine   | Dimethylpyridine     |
| Morpholine            | Dimethylethylpyrrole |
| Pyridine              | Piperazine           |

The additive is interground with the mineral in the grinding mill to provide increased grinding efficiency as well as other advantageous results, e.g., inhibiting pack set of bulk stored materials or inhibiting the formation of foam in some mineral processing applications. It has also been found that the novel additive of the present invention also serves to provide fluidity to the ground minerals when they are being transported by conveying systems, particularly by pneumatic air systems.

The term "mineral" as used herein is intended to refer to naturally occurring inorganic minerals, such as phosphate rock, partially processed minerals such as concentrated iron ore, and mixtures of minerals such as cement clinker or ceramics.

Further examples of such minerals which can be processed with the additive of the present invention, mention may be made of beryllium oxide, limestone, gypsum, clays, and bauxite.

The additive of the present invention is particularly

preferred for use with cement, and cement-forming materials particularly portland cement.

Portland cement represents a class of hydraulic cements and is comprised essentially of two calcium silicates and a lesser amount of calcium aluminate. These cements are produced by heating an intimate mixture of finely divided calcareous material (limestone) and argillaceous material (clay) to fusion to form a clinker. The clinker is ground with the addition of about 5% gypsum, or some other form of calcium sulfate, to obtain the desired setting qualities in the finished cement. It is to the clinker that the novel additive of this invention is preferably added to increase grinding efficiency and to inhibit subsequent pack set in the finished cement.

The additives of the present invention are employed in either dry or liquid form. For convenience, the additive is in liquid form to permit accurate metering into the mineral stream. In instances where the additive is not very soluble in water, it can be utilized by emulsifying it with a suitable wetting agent, e.g., sodium dodecyl benzene sulfonate. The addition is accomplished either prior to the grinding or the additive is introduced into the grinding mill simultaneously with the mineral. If the additive is employed merely for reduction of pack set and fluidizing purposes, it is added at any convenient point in the processing.

The additive of the present invention is employed as the sole grinding aid or with a mixture of one or more grinding aids or with additives known to the art other than grinding aids, e.g., set retarders or accelerators, in the case of cement.

The additive is employed effectively over a relatively wide range. The preferred range is about 0.001 to 1%, and more preferably about 0.005 to about 0.1% based on the weight of the mineral, i.e., weight of additive solids based on weight of mineral solids (herein referred to as solids on solids). In a particularly preferred embodiment about 0.05% of the additive based on the weight of the mineral is employed. The higher levels are employed if grinding to a relatively high surface area, and the amount of additive used is limited only by the desired surface area and fluidity of the finished product.

In Table 1 the effectiveness of the additives as grinding aids is reported. The data reported was obtained using a Type 1 cement clinker and gypsum ground in a laboratory mill at a temperature of 210° F. for 7411 mill revolutions.

TABLE 1

| Additive           | Amount of additive (percent solid on solid) | Blaine surface area, cm. <sup>2</sup> /g. |
|--------------------|---------------------------------------------|-------------------------------------------|
| Blank              |                                             | 3,441                                     |
| Aniline            | 0.01                                        | 3,503                                     |
| Do                 | 0.05                                        | 3,660                                     |
| Morpholine         | 0.01                                        | 3,480                                     |
| N-methylmorpholine | 0.01                                        | 3,500                                     |
| P-toluidine        | 0.01                                        | 3,570                                     |
| Pyrrolidine        | 0.01                                        | 3,542                                     |
| Do                 | 0.05                                        | 3,515                                     |
| Piperidine         | 0.01                                        | 3,499                                     |
| Diphenylamine      | 0.01                                        | 3,550                                     |

In Table 2, pack set data is reported on cement inter-ground with the additives of this invention.

TABLE 2

| Additive           | Addition rate (percent solid on solid) | Pack set index |
|--------------------|----------------------------------------|----------------|
| Blank              |                                        | 12.6           |
| Aniline            | 0.05                                   | 10.0           |
| Morpholine         | 0.01                                   | 11.3           |
| Do                 | 0.05                                   | 2.0            |
| N-methylmorpholine | 0.01                                   | 11.3           |
| P-toluidine        | 0.01                                   | 12.3           |
| Do                 | 0.05                                   | 4.0            |
| Pyrrolidine        | 0.01                                   | 8.0            |
| Do                 | 0.05                                   | 1.0            |
| Piperidine         | 0.01                                   | 9.0            |
| Diphenylamine      | 0.05                                   | 7.3            |

In a particularly preferred embodiment the additive employed is morpholine and morpholinyl derivatives. Various grades and purities of the morpholine compounds are employed with satisfactory results. A particularly preferred source of morpholine type compounds is a byproduct from the continuous commercial production of heterocyclic amines. The by-product contains a mixture of aliphatic and heterocyclic mono- and diamines. The morpholinyl ring, however, is the dominant group present.

Table 3 shows a typical analysis of a by-product which is predominantly a mixture of 4-(2-aminoethoxy) ethylmorpholine, 2-(4-morpholylethoxy) ethanol and bis-2-(4-morpholinyl) ethyl ether.

Table 3

|                             |       |             |       |
|-----------------------------|-------|-------------|-------|
| Titratable amine            | ----- | Meq./g.     | 7.52  |
| Primary amine               | ----- | Meq./g.     | 1.66  |
| Tertiary amine              | ----- | Meq./g.     | 4.57  |
| Total nitrogen              | ----- | Meq./g.     | 7.93  |
| Total acetylatable material | ----- | Meq./g.     | 7.02  |
| Specific gravity            | ----- | 20/20° C    | 1.078 |
| Water content               | ----- | wt. percent | 0.08  |

In Table 4 the grinding efficiency and pack set data of the additive of Table 3 is reported. The data was collected using a Type I cement clinker and gypsum ground in a laboratory mill at 210° F. for 7411 mill revolutions.

TABLE 4

| Amount of additive (percent solid on solid) | Blaine surface area, cm. <sup>2</sup> /g. | Pack set index |
|---------------------------------------------|-------------------------------------------|----------------|
| Blank                                       | 3,441                                     | 12.6           |
| 0.05                                        | 3,605                                     | 1.0            |

From the above table it can be seen that the use of even a very small amount of additive results in an increase in grinding efficiency of about 164 units as well as a substantial decrease in pack set index.

The novel additive described in Table 3 was also used to grind phosphate rock. After grinding phosphate rock with 0.03% of the additive described in Table 3 in a laboratory mill for 3752 revolutions at 200° F., 61% of the ground product passed a 200 mesh screen whereas only 54% of a control sample (no additive) passed a 200 mesh screen.

In addition to using the above described amine compounds per se as mineral additives, the reaction product of the amines and an aliphatic organic acid having 2 to 20 carbon atoms are also employed as additives and provide enhanced grinding efficiency. The product is prepared by the addition of acid, preferably glacial acetic acid to cause the pH to drop to not less than about 7. In a preferred embodiment the pH is lowered to about 8. The acetylated amine acetate is produced by the addition of acid anhydride to the amine instead of the acid.

The following table illustrates the use of the reaction product of the amine described in Table 3 and acetic acid (pH 8) in grinding cement clinker. The Type 1 cement clinker and gypsum were ground for 4095 revolutions in a laboratory mill heated to 200° F.

TABLE 5

| Amount of additive (percent solid on solid) | Blaine surface area (cm. <sup>2</sup> /g.) | Pack set index | Air entrainment |
|---------------------------------------------|--------------------------------------------|----------------|-----------------|
| Blank                                       | 3,590                                      | 6              | 10.0            |
| 0.058                                       | 3,850                                      | 0              | 10.3            |

From Table 5 it can be seen that the grinding efficiency and pack set properties are increased and no air is entrained.

As stated above, the present invention is also directed to mixtures of additives. A particularly preferred mixture is prepared from the amine described in Table 3, triethanolamine and acetic acid. A preferred source of triethanolamine is the residue product obtained in production of ethanolamines. The exact composition of the residue product varies within certain limits and, there-

fore the residue product may contain one or more of mono-, or diethanolamine in addition to the triethanolamine. One such residue product has the following analysis before neutralization.

TABLE 6

|                   |                   |            |
|-------------------|-------------------|------------|
| Triethanolamine   | percent by volume | 45 to 55   |
| Equivalent weight |                   | 129 to 139 |
| Tertiary amine    | meq./gm.          | 6.2 to 7.0 |
| Water             | by weight, max.   | 0.5        |
| Density           | lbs./gal.         | 9.49       |

The following table illustrates the grinding efficiencies obtained using the reaction product of acetic acid and a 50-50 (by weight) mix of the amines of Table 3 and Table 6. The pH of the mixture was 8. Type I cement clinker and gypsum were ground in a laboratory mill at 220° F.

TABLE 7

| Amount of additive<br>(percent solid on solid) | Mill<br>revolutions | Blaine surface<br>area, cm. <sup>2</sup> /g. | Pack set index |
|------------------------------------------------|---------------------|----------------------------------------------|----------------|
| Blank                                          | 7,558               | 4,270                                        | 55             |
| 0.012                                          | 7,343               | 4,330                                        | 6              |
| 0.018                                          | 7,343               | 4,400                                        | 7              |
| 0.025                                          | 6,587               | 4,300                                        | 3              |

Another additive mix which is particularly useful in the present invention is one which contains 60% of the additive mix whose grinding data is described above in Table 7, 20% urea and 20% water. Table 8 shows the grinding data achieved by such a mixture when Type 1 cement clinker and gypsum are ground in a laboratory mill for 5092 revolutions at 220° F. with the additive used at a level of 0.04% (solid on solid).

TABLE 8

|          | Blaine surface<br>area, cm. <sup>2</sup> /g. | Pack set index |
|----------|----------------------------------------------|----------------|
| Blank    | 3,250                                        | 38.0           |
| Additive | 3,599                                        | 1.5            |

The above additive has the additional advantage of not becoming unduly viscous at low temperatures.

While the additive of the present invention has been described primarily in terms of grinding cement clinker and phosphate rock, satisfactory results are obtained when the additive is utilized in grinding other minerals as described above.

What is claimed is:

1. A composition comprising a mineral and from 0.001 to 1 weight percent of an additive intimately admixed

therewith, the said additive being compounds selected from the group consisting of morpholine, N-methylmorpholine, and a byproduct from the continuous commercial production of heterocyclic amines consisting predominantly of 4-(2-aminoethoxy) ethylmorpholine, 2-(4-morpholethoxy) ethanol, and bis-2-(4-morpholiny) ethyl ether.

2. A composition comprising a mineral and intimately admixed therewith, from 0.001 to 1% based on the weight of the mineral of a mixture of (1) an aliphatic organic acid having 2-20 carbon atoms, (2) a residue product of ethanolamine synthesis, and (3) a compound selected from the group consisting of morpholine, N-methylmorpholine, and a byproduct from the continuous commercial production of heterocyclic amines consisting predominantly of 4-(2-aminoethoxy) ethylmorpholine, 2-(4-morpholethoxy) ethanol, and bis-2-(4-morpholiny) ethyl ether, said residue product being predominantly triethanolamine and having the following properties before neutralization:

Triethanolamine ----- 45 to 55% by volume  
Equivalent weight ----- 123 to 139  
Tertiary amine ----- 6.2 to 7.0 meq./gm.  
Water ----- 0.5% by weight, max.  
Density ----- 9.49 lbs./gal.

the proportions of (2) and (3) being equal parts by weight, and the proportion of acid being sufficient to bring the pH of the mixture to 8.

3. The composition of claim 1 wherein the mineral is portland cement.

#### References Cited

#### UNITED STATES PATENTS

|           |         |               |         |
|-----------|---------|---------------|---------|
| 2,857,286 | 10/1958 | Striker       | 106—102 |
| 3,042,718 | 7/1962  | Evans et al.  | 252—384 |
| 3,088,837 | 5/1963  | Prescott      | 106—308 |
| 3,278,269 | 10/1966 | Ekker         | 252—384 |
| 3,305,491 | 2/1967  | Oster         | 252—384 |
| 3,325,105 | 6/1967  | Veltman       | 106—102 |
| 3,329,517 | 7/1967  | Dodson et al. | 106—315 |

TOBIAS E. LEVOW, Primary Examiner.

SAMUEL E. MOTT, Assistant Examiner.

#### U.S. Cl. X.R.

106—102, 315; 241—16; 252—384